

Aug. 4, 1936.

F. C. ELDER

2,049,834

MANUFACTURE OF HOT GALVANIZED ARTICLES

Filed Dec. 9, 1935

Fig. 1.



Fig. 2.



Fig. 3.



Inventor:

Flinch C. Elder  
by Maria Rauher  
-his Attorneys.

## UNITED STATES PATENT OFFICE

2,049,834

## MANUFACTURE OF HOT GALVANIZED ARTICLES

Flint C. Elder, Cleveland Heights, Ohio

Application December 9, 1935, Serial No. 53,510

16 Claims. (Cl. 91—70.2)

This invention relates to the manufacture of coated metal articles, and while not limited thereto relates more particularly to the manufacture of hot galvanized or zinc coated ferrous metal articles; such as iron rods, wires, strips and sheets. The invention of the present application is a continuation in part of that shown and described in my copending application, Serial No. 692,684 filed October 7, 1933.

Heretofore, in the coating of metal articles with dissimilar metals, and particularly in the galvanizing of ferrous articles, it has been the practice to immerse the article to be coated in a bath of molten zinc for such a period of time as is necessary to alloy the coating metal to the superficial areas of the base metal. Upon withdrawal from the coating bath, the coated article will be found to have, in general, three distinct metallic constituents in superimposed relation when viewed in cross-section. The innermost portion of the article will, of course, be the base metal. Superimposed thereon will be a thin alloy layer, or layers, of the coating metal combined with the base metal.

In the case of a ferrous base metal and a zinc coating, this alloy layer, or layers, will be iron-zinc compounds represented, for the most part, by the chemical symbols,  $FeZn_3$  and  $FeZn_7$ . Superimposed atop this alloy layer will be a stratum of pure coating metal, or zinc, which will have adhered to the article upon its withdrawal from the bath, and which will have become frozen thereon upon being exposed to the air to constitute the outermost layer and surface of the coated article.

Where it has been deemed desirable to increase the coating upon the base metal, according to prior art methods, the coated article has been returned to the same, or to a similar, coating bath for re-immersion therein. The temperatures of the secondary bath, and the length of time of immersion, have been such as to materially increase the total bulk of the coated articles. However, analysis of the final product has clearly indicated that the total increase in weight of coating in every instance has been accompanied by a growth of the alloy layer, and that the outer layer of pure coating metal, is not increased appreciably over the initial coating.

It was found that the coatings on such articles, when coated in accordance with methods heretofore known, possess low ductile properties and brittleness, resulting in cracking and failure of the coating when subjected to the

flexing and bending stresses occasioned by average usage. The cause for this undesirable brittleness has been definitely ascribed to the alloy strata of the articles coated as above described; particularly where one prolonged immersion or two or more immersions are made in an effort to increase the coating. Such increase of the time of immersion has always resulted in a material increase of the alloy strata without contributing to the thickness of the outer layer of pure coating metal.

It is apparent from the above discussion that it is highly desirable to acquire a coating upon a base metal composed almost entirely of the pure coating metal; such as zinc, wherein the alloy layer intermediate the base metal and the pure coating metal is held to the irreducible minimum of that formed by the initial dip in the conventional way. The alloy layer formed from such an initial dip is not of sufficient magnitude to impair the physical properties of the coating on the coated article. However, subsequent immersions in a molten coating bath in the conventional way do cause an increase in the alloy layer on the coated article to thereby seriously impair the physical properties of the coating.

The principal object of this invention is to provide a novel method of manufacturing hot galvanized or zinc coated metal articles, whereby a materially heavier coating will be formed on the articles than has heretofore been possible of production by hot galvanizing in accordance with prior art methods.

Another object of this invention is to provide a novel method of manufacturing hot galvanized or zinc coated metal articles whereby the zinc coating will have a materially greater thickness of relatively purer zinc than has heretofore even been considered possible in hot galvanizing.

Still another object is to produce coated articles having a heavy, pure coating of a metal thereon, which coating will be homogeneous, strong and possessed of good ductility and excellence of finish.

In the manufacture of hot galvanized or zinc coated articles the article to be galvanized is prepared for the galvanizing step by cleaning the surface of the article, fluxing the article, then passing the so prepared article into and through a molten bath of high grade relatively pure zinc.

The article passing from the bath of molten zinc has a coating composed of an alloy of the

base metal and the zinc next to the base metal and an outer layer of substantially pure zinc. The amount of coating; that is, the thickness of coating on the metal article, has heretofore been 5 regulated by the time of immersion of the article in the bath, either in one or more immersions.

In order to make a specific disclosure of this 10 invention it will be described as applied to the manufacture of hot galvanized or zinc coated iron or steel wire, it being understood that by a slight modification the same process may be applied to other metal articles in the form of strips, sheets, bars or shapes.

15 In the general method of galvanizing iron or steel wire the wire or rod is run successively through an acid cleaning bath, water washing bath, fluxing bath, and then into a bath of molten high grade or substantially pure zinc 20 from which it emerges through a suitable wiper and then is wound upon a standard take-up block. The temperature of the molten zinc forming the bath through which the wire rod to be coated is passed is commonly carried at 25 300 to 900 degrees Fahrenheit. The amount of coating applied to the wire or rod has heretofore been regulated solely by the time of immersion of the wire or rod in the zinc bath; that is, by the length of immersion and the speed at which the wire rod travels through the bath.

Increasing the length of time of immersion of the wire rod or other article in the molten zinc bath increases the amount of thickness of the 35 coating obtained on the wire rod within well defined limits, since in actual operation it is recognized that after a predetermined time of immersion there is substantially no further increase of the amount of coating obtained. Experience has shown that a #12 gage (.1055") diameter iron or steel wire regardless of the increase in the length of time of immersion will not receive a single coating greater than that equal to approximately 1.25 ounces of coating 40 45 per square foot of wire surface. If this same wire is re-galvanized in accordance with the usual practice, except for omitting the acid cleaning, the wire will be found to retain substantially the same weight of pure coating as resulted in the first galvanizing. In other words, experience has shown that doubling the 50 55 total time of immersion or re-immersing galvanized wire, rods and the like causes no appreciable increase in the weight of pure galvanized coating.

The present invention provides for increasing the weight of zinc or galvanized coating on wire, rods and the like far beyond that heretofore thought possible.

60 In the drawing:

Figure 1 shows a diagrammatic elevation of apparatus in carrying out the method of the invention.

Figure 2 shows a slightly modified form of 65 apparatus in carrying out the invention.

Figure 3 shows a cross-section through a wire or rod coated in accordance with the invention.

In carrying out the method of this invention the wire, rod or other material A, as desired or necessary, is annealed by passing it continuously 70 through the annealing furnace 2. As the material exits from the furnace 2 it is passed continuously through an acid bath contained in a vat 3, then through a washing vat 4, containing 75 wash water, and then through the flux in a

fluxing tank 5, thence through a molten zinc bath contained in the zinc pan 6. The zinc pan 6 is provided with a burner 7 at its entrance end which maintains the zinc bath molten, and the portion of the bath closest to said burner is of materially higher temperature than the portion of the bath farthest away from said burner. The material A to be coated enters the molten zinc or galvanizing bath at its hottest point, substantially above the burner 7, and 10 travels through the bath at such a speed and for such a distance as to remain in the bath a sufficient length of time to cause an alloying of the zinc and the metal to be coated, and the accumulation of the maximum amount of 15 substantially pure zinc coating surrounding the so formed alloy layer. The wire, rod or other article to be coated exits from the molten zinc bath and travels continuously in the atmosphere for a sufficient length of time to cause the zinc 20 coating to freeze. After the coating is frozen or solidified the coated wire or rod is successively passed at intervals into the relatively cool end of the galvanizing or zinc bath to increase the weight of coating. In the drawing the wire 25 or rod is shown as passing from the galvanizing or zinc bath in the pan 6 upwardly over a sheave or roll 8, then downwardly into the zinc bath and around a sheave or roll 9 immersed in the zinc bath, then upwardly and over a 30 sheave or roll 10 located materially above the pan 6, and then downwardly through the molten zinc or galvanizing bath under a sheave or roll 12, thence outwardly over a suitable guide sheave 14 to a take-up reel 15. 35

If desired, it will be understood that even more successive passes may be made through the molten zinc bath to further increase thickness of the zinc coating. The successive passes of the coated metal through the molten zinc bath 40 are accomplished with great rapidity and are for relatively short intervals only, whereby additional substantially pure zinc is applied to the coating to materially increase its weight and thickness and while the alloy portion of the 45 coating remains substantially unchanged. It is desirable that the successive passes of the coated article after the first coating is formed be made in a molten zinc bath of materially less temperature than the zinc bath into which the un-coated base metal enters, although this is not 50 necessary.

It will be understood that the nearer the melting point the molten bath can be maintained the less critical the control over the amount of coating acquired in the second bath becomes. This is explained by the fact that the heat of such a bath is insufficient to cause even the superficial areas of the initial coating to melt, whereby the initial coat is preserved in its entirety. The 60 hotter the baths succeeding the initial bath are, the more rapid must be the immersions of the pre-coated base metal therein to prevent the melting off of the pre-coat, and, hence, the results become even more difficult of predetermination. However, it will be understood that a heavy, substantially pure coating may be formed in a bath of even higher temperature than preceding baths, provided that the duration of immersion is proportionately diminished, 65 and/or provided that the precoated base metal has been proportionally chilled before immersion.

In Figure 2 the modified apparatus for carrying out this invention is substantially the same as that described above, with the exception that 75

the galvanizing pan has been modified. The same reference numerals will be applied to like parts of the apparatus of Figure 2. The galvanizing pan of Figure 2 is designated by the 5 numeral 6<sup>a</sup>. The pan 6<sup>a</sup> is divided into two chambers X and Z, by a partition wall 20 so as to prevent circulation of the molten zinc from the one chamber to the other. Material to be coated enters the chamber X of the pan 6<sup>a</sup> and 10 passes through this chamber, then out over the guide roll or sheave 8<sup>a</sup> and down under a guide sheave or roll 9<sup>a</sup> in the chamber Z. From under the roll 9<sup>a</sup> the metal passes upwardly through the atmosphere and over a guide sheave 15 or roll 10<sup>a</sup>, thence downwardly under a guide roll or sheave 12<sup>a</sup>, and over a guide sheave or roll 14 to the usual take-up block, as described for the apparatus in Figure 1.

Experience has shown that in carrying out the 20 method of this invention, with apparatus similar to that described above, the relatively short immersions of the coated article in the molten bath of zinc having a less temperature than that normally maintained for galvanizing, causes a 25 material increase after each immersion in the weight and thickness of the relatively pure zinc coating on the article. The zinc bath in which the successive short immersions are made is preferably maintained at a temperature as near 30 to the melting point of zinc as is practical, and with successive immersions for length of time in the order of less than one second for #12 gage wire, the relatively pure zinc coating can be increased to practically any desired amount.

35 In coating wire according to the present invention, I have placed almost 10 oz. of zinc per square foot of wire surface on a #12 gage iron wire, and have maintained the ferrous content of that coating to below 1% by weight. This 40 is over four times the amount of zinc coating acquired by prior art methods on the same gage wire fabricated in accordance with the customary practice on competitive articles.

As a specific example, #12 gage steel wire has 45 been coated, using a zinc or spelter temperature of 840 to 850 degrees Fahrenheit at the entering end of the galvanizing pan, and a length of immersion in the zinc bath to form the initial coating of approximately one minute. The resultant initial coating had a maximum weight 50 of approximately 1.25 ounces per square foot of wire surface. An additional immersion of the initial galvanized wire in the spelter bath having a temperature approximately at the melting 55 point of the zinc for one second caused an increase in weight of the galvanizing or zinc coating of considerably more than five ounces per square foot of wire surface, and additional short immersions caused a similar increase in the 60 relatively pure zinc coating, without appreciably increasing the alloy constituency.

While the exact theory on which this invention is based is not certain, it is a generally accepted fact that hot galvanized wire, rod or 65 other article has at least three different layers in the coating, as illustrated in Figure 3 of the drawing; that is, next to the base metal there is a high iron content or ferrous zinc alloy, designated in the drawing as 30, and on the outside 70 of this iron or ferrous zinc alloy is the second alloy layer of lower iron content and more correctly termed a zinc iron or ferrous zinc alloy, which is designated in the drawing by the numeral 31. The third or surface layer of the zinc immersed or galvanized wire, rod or other

75 article is composed of substantially pure zinc, as designated in the drawing by the numeral 32.

Heretofore, the three layers above described formed the complete coating. The two innermost alloy layers are relatively thin in comparison with the outer relatively pure zinc layer, and because of their iron or ferrous content the inner layers have a melting point considerably higher than the outer or pure zinc layer. The alloy layers are, therefore, in a 10 solid condition while the pure top layer is in a molten condition as a galvanized wire or article emerges from the galvanizing bath. The generally accepted theory is that the amount of 15 pure zinc in the outer layer is practically constant with a fixed bath temperature and speed, but the two alloy layers increase materially with time of immersion, the rate of increase becoming progressively slower as the alloy layers increase in thickness since the zinc has to diffuse 20 through the solid alloy layers. The alloy layers are solid because their melting points are higher than the bath temperature commonly carried in galvanizing.

The amount of the outer relatively pure layer 25 of zinc galvanizing depends on the amount of liquid or molten zinc carried on the wire as it passes from the bath, and this amount of zinc depends on the fluidity of the bath, the lower the temperature within limits the more galvanizing or zinc will be carried out of the bath on the article frozen thereon.

In the present process the initial coating is allowed to freeze and then the so-coated article or wire is returned to the bath (either the same 35 bath or a second one) and allowed to remain in the bath for a length of time only sufficient to permit additional molten metal to freeze upon the initial coating without melting it and the article is then immediately withdrawn from 40 the bath.

Examination of the article upon withdrawal 45 from the bath after the second dip has disclosed that no bond is formed between the first and second coatings. In the case of wire, the second coating resembles a zinc pipe shrunk upon the pre-coated wire or base metal. It has been deduced from this that the pre-coated base metal, when introduced into a bath of molten zinc, rapidly absorbs the heat from that portion of the 50 zinc bath immediately surrounding and near it, thereby actually causing a mass of zinc to freeze upon it while still in the bath. Thereafter, the coated article is immediately withdrawn before it can become saturated with the heat of the 55 bath; i. e., before its refrigerating effect is neutralized, whereby the zinc coating thus formed is retained in toto without melting off. Thus, it will be clearly seen that if no bond is formed between the first and subsequent coatings there 60 can be no melting of the first coating. This is significant because of two reasons; first, the entire initial coating is preserved without loss. In this connection I have found that such heat required to melt even the superficial areas of 65 the initial coating will cause that coating to run off entirely. Hence, even if bonding can be theoretically effected by this method, it is so extremely critical as to be uncontrollable as a practicable matter. Secondly, if the initial 70 coating is not melted, nor heated to melting point, then obviously, as above noted, there can be no increase of the undesirable alloy constituency. Additional immersions may be made until the desired weight of coating has been built up 75

on the article, and it will be found that the alloy layer of the initial coating will show no apparent increase from such successive short immersions. The coated article or wire is preferably allowed to cool between the successive coating steps to a temperature appreciably below the melting point of zinc.

Referring again to the drawing it will be noted that the layer of relatively pure zinc 32 formed by the initial coating is less than twice the thickness of the combined alloy layers 30 and 31, and that successive layers of relatively pure zinc, 33 and 34, which result from successive short immersions as described heretofore, 15 are substantially the same thickness or greater than that of the pure zinc layer of the initial coating.

After an article has been coated in accordance with the method outlined herein, I provide that 20 it shall be worked, either hot or cold, in any suitable manner, as by rolls, drawing dies, etc. This final working not only serves to refine the grain structure of the coatings and to improve the finish or luster thereof but also effects a 25 complete coalescence between the several coatings to make them into one, integral, homogeneous coating. All tendency of the coating to crack or flake off when flexed or distorted in use is thereafter precluded.

30 It will be seen from the above description that my method applies to cases where it is desirable to place a substantially pure coating of one metal upon another without permitting the growth of an undesirable alloy stratum between the two. Obviously, then, my invention relates to the coating of any article that has an initial coating of the same metal already formed thereon, as well as to those uncoated articles which receive the initial coating in accordance 35 with the conventional practices recited herein. Therefore, my invention is equally applicable to articles pre-coated in any way, as by electrolytic deposition, spraying, flowing, extrusion, etc. Hence, any of the conventional coating processes 40 may be substituted for the initial dip step disclosed herein merely for purposes of illustration.

To recapitulate my invention, I take an article to be coated in accordance herewith, which either has an initial coating alloyed thereto or 45 upon which I form such a coating in any suitable way. After the initial coating has thoroughly set, I increase that coating by rapidly dipping the article into a molten bath of the same metal, and instantly withdrawing it before the initial coat can be melted or otherwise dissipated. Successive rapid dips of only a second or less in duration may be made to still further increase the thickness of the coating any desired amount.

50 While I have shown and described certain specific embodiments of my invention it is to be understood that I do not wish to be limited exactly thereto, since various modifications may be made 55 without departing from the scope of my invention, as defined by the following claims.

I claim:

1. The method of forming an integral, homogeneous coating upon an article having a pre-formed coating of a given metal alloyed thereto 60 which includes rapidly dipping said article in a molten bath of said given metal to acquire a covering thereof without melting or otherwise affecting said preformed coating, permitting the 65 second coating to set, and thereafter treating

the coated article to effect coalescence between the coatings.

2. The method of forming an integral, homogeneous coating upon an article which includes alloying a solid coating of a given metal thereon, subsequently immersing the initially coated article in a bath of said given metal and instantly withdrawing the same to acquire a secondary coating without melting the solid coating, and thereafter treating the coatings to effect coalescence therebetween. 10

3. The method of covering an article with a relatively pure, heavy coating of a given metal which includes bonding a coating of said given metal to the article to be coated, and thereafter 15 rapidly dipping the coated article in a molten bath of said given metal to acquire a substantial covering thereof upon the initial coating without melting or otherwise affecting the integrity of the initial coating. 20

4. The method of covering an article with a relatively pure, heavy coating of a given metal which includes bonding a coating of said given metal to the article to be coated, permitting the bonded coating to set, rapidly dipping the coated 25 article in a molten bath of said given metal to freeze an unbonded layer thereof upon said coated article, and thereafter treating the article so coated to integrate said bonded coating and unbonded layer into a single homogeneous coating. 30

5. The method of increasing the coating upon a base metal having an initial coating of a given metal bonded thereto which includes rapidly dipping said pre-coated base metal in a molten bath of said given metal to acquire a coating thereof 35 upon the initial coating without affecting the integrity of said initial coating.

6. The method of increasing the coating upon a base metal having an initial coating of a given metal bonded thereto which includes rapidly dipping 40 said pre-coated base metal into a molten bath of said given metal to form an unbonded additional coating thereon without affecting the integrity of said initial coating, and thereafter treating said coatings to integrate the same. 45

7. The method of continuously coating metallic articles with a given metal which includes bonding a coating of said given metal upon the articles to be coated and thereafter rapidly dipping said articles at least once in at least one 50 molten bath of said given metal to form a plurality of coatings on said articles without affecting the next preceding coating, and thereafter treating said articles to completely integrate said coatings and to improve the finish and physical 55 properties thereof.

8. The method of galvanizing articles which includes rapidly dipping an article having a pre-formed coating of zinc bonded thereto into a molten bath of zinc to acquire a substantial additional coating thereof upon the preformed coating without affecting the integrity of said pre-formed coating. 60

9. The method of hot galvanizing articles which includes rapidly dipping an article having a pre-formed coating of zinc bonded thereto at 65 least once in at least one bath of molten zinc to acquire a substantial additional coating thereof without affecting the integrity of the preceding coating, and thereafter treating said article 70 to integrate all coatings, each coating in turn being permitted to completely set before being introduced to the next succeeding step of the method.

10. As an article of manufacture a metallic 75

article having an integral homogeneous coating formed thereon by the hot-dip method in excess of 2.5 oz. per square foot of surface and with an impurity content of less than 1% by weight.

5 11. As an article of manufacture a metallic article having a hot-dipped coating thereon in excess of 2.5 oz. per square foot of surface, said coating being integral, homogeneous and bonded to said article.

10 12. As an article of manufacture a metal article having a hot-dipped zinc coating bonded thereto in excess of 2.5 oz. per square foot of surface, said coating being substantially pure, integral and homogeneous.

15 13. The method of coating attenuated metal stock which includes passing said stock through a bath of molten metal and alloying a coating of the bath metal thereon, permitting said coating to solidify, and thereafter rapidly passing said coated stock through a bath of said molten metal to acquire a relatively heavy coating thereof

upon said initial coating without affecting the integrity of the latter.

14. The method of hot-galvanizing attenuated metal stock which includes passing said stock through a bath of molten zinc to alloy a coating of zinc thereon, permitting said zinc coating to solidify, and thereafter rapidly passing said coated stock through a bath of molten zinc to acquire a relatively heavy coating thereof upon said initial coating without affecting the integrity of the latter.

15. The invention recited by claim 13 which further includes treating the coated stock to integrate said coatings, and to improve the physical characteristics and finish thereof.

16. The invention recited by claim 14 which further includes treating the zinc-coated stock to integrate said coatings, and to improve the physical characteristics and finish thereof.

20 FLINT C. ELDER.